



The products described herein can be used in oils in amounts of 0.1% to 40% by weight, preferably 0.1% to 15%; more preferably, 1% to 10%.

The following examples illustrate the formation of the reaction product useful herein as corrosion inhibitors and detergents in lubricating oil compositions.

#### EXAMPLE I

A mixture of 51 grams (0.23 mol) of phosphorus pentasulfide, 500 grams of an oil solution of N-butyl polyisobutyl succinimide (0.21 mol), wherein the polyisobutyl radical contained an average of approximately 66 carbon atoms, and 500 grams of xylene was heated at reflux temperatures for a period of 5 hours under a blanket of nitrogen. The xylene was distilled off under reduced pressure (310° F. bottoms temperature at 4 mm.). For convenience the product is called Product A.

A mixture of 250.12 grams of Product A and 16.0 grams of tetraethylene pentamine was heated to 150° F., using a blanket of nitrogen over the reaction mixture. The mixture was slowly heated to 350° F. at an absolute pressure of 4 mm. Hg, and heated at that temperature and pressure for 2 hours.

The reaction product contained:

|            | Wt. percent |
|------------|-------------|
| Phosphorus | 2.54        |
| Sulfur     | 3.21        |
| Nitrogen   | 2.64        |

#### EXAMPLE II

A mixture of 137.6 grams (0.62 mol) of phosphorus pentasulfide, 2700 grams (1.24 mols) of an oil solution of N-butyl polyisobutyl succinimide, and 2700 grams of xylene was heated at reflux temperature for 5 hours. The xylene was removed by heating the mixture at 310° F. at an absolute pressure of 4 mm. Hg. The remaining product was dissolved in hexane and filtered, and the hexane was removed.

A mixture of 2600 grams of the above product and 166 grams of tetraethylene pentamine was heated to 150° F., followed by heating at 350° F., at an absolute pressure of 4 mm. Hg for 2 hours.

The reaction product contained:

|            | Wt. percent |
|------------|-------------|
| Phosphorus | 1.30        |
| Sulfur     | 1.26        |
| Nitrogen   | 2.60        |

#### EXAMPLE III

A mixture of 184 grams (0.83 mol) phosphorus pentasulfide, 1600 grams (0.73 mols) of an oil solution of N-butyl polyisobutyl succinimide, and 1200 ml. benzene was heated at reflux temperature under a blanket of nitrogen for 30 minutes. The reaction mixture was filtered, and the benzene was removed by distillation.

A mixture of 200 grams of the above product and 12.8 grams of tetraethylene pentamine was heated to 150° F., then to 350° F. at an absolute pressure of 4 mm. Hg.

The final product contained:

|            | Wt. percent |
|------------|-------------|
| Phosphorus | 1.06        |
| Sulfur     | 0.88        |
| Nitrogen   | 2.65        |

Table I hereinbelow presents further data on the effectiveness of the reaction products described herein as lubricating oil additives. The data of Table I were obtained after 60 hours of operating under the severe conditions of a Caterpillar 1-H engine test used to qualify oils under the Mil 2104B procedure. This military specification procedure is so severe that the engine will not even operate with a base oil uncompounded. Even a base oil with the normal commercial additives under this procedure does not provide sufficient lubrication; that is, the engine itself eventually sticks.

The base oil used in obtaining data for Table I con-

sisted of a California paraffinic base oil having a viscosity of 500 SSU at 100° F., and having incorporated therein 15 mM./kg. (i.e., 15 millimols of metal per kilogram of the finished lubricating oil composition) of a basic sulfurized calcium phenate, and 12 mM./kg of a zinc dialkyl dithiophosphate.

The "PD Nos." refer to the piston discoloration rating. After the engine test, the three piston lands are examined visually. To a piston land which is completely black is assigned a PD No. of 800; to one which is completely clean, a PD No. of 0; to those intermediate between those completely black and completely clean are assigned PD Nos. intermediate in proportion to the extent and degree of darkening.

The "GD No." refers to the percentage deposit in the top piston ring groove; that is, a 0 evaluation being a clean groove, and a 100 evaluation being a groove full of deposits.

Table I

| Composition                                | Hrs.        | PD Nos.                        | GD No.  | Break-in-Wear, mgs. loss |
|--------------------------------------------|-------------|--------------------------------|---------|--------------------------|
| 1. Base Oil + 4% wt. Product of Example I  | { 60<br>120 | 245-140-110-5<br>305-190-135-5 | 8<br>13 | 199<br>336               |
| 2. Base oil + 4% wt. Product of Example II | { 60<br>120 | 200-65-145-0<br>215-120-140-0  | 6<br>11 | 296<br>487               |

Table II hereinbelow presents data showing the effectiveness of the compounds described herein as lubricating oil additives by testing a lubricating oil composition in an L-38 Test, using a 1 cylinder CLR engine in a test period of 40 hours.

The base oil consisted of a California paraffinic base oil having a viscosity of 500 SSU at 100° F., 14 mM./kg. of a zinc dialkyl dithiophosphate, and 4 mM./kg. of a zinc di(alkylphenyl) dithiophosphate.

Table II

Bearing weight loss (milligrams)

Composition: (1) Base oil + 6.25% of product of Example II

310

Table III hereinbelow presents data obtained with lubricating oil compositions containing the reaction product of Example II hereinabove.

The test was made in a Caterpillar L-1 engine according to the Supplement I conditions (for a period of the hours noted) as described in the Coordinating Research Council Handbook, January 1946.

The "PD Nos." and "GD Nos." are defined hereinabove.

The base oil was a Mid-Continent SAE 30 oil containing 10 mM./kg. of a zinc dialkyl dithiophosphate, and 2 mM./kg. of a zinc di(alkylphenyl) dithiophosphate.

Table III

| Composition                             | Hours       | GD Nos. | PD Nos.        |        |
|-----------------------------------------|-------------|---------|----------------|--------|
|                                         |             |         | Land           | Skirt  |
| 1. Base Oil + 2% Product of Example III | { 60<br>120 | 1<br>1  | 5-0-0<br>5-0-0 | 0<br>0 |

In addition to the additives described hereinabove, the lubricating oils herein may contain other corrosion inhibitors, oxidation inhibitors, thickening agents, viscosity index improving agents, rust inhibitors, etc.

We claim:

1. A lubricating oil composition comprising a major proportion of a lubricating oil having incorporated therein from 0.1% to 40% of a product obtained by (1) reacting an N-alkyl alkenyl succinimide having from 30 to

200 carbon atoms in said alkenyl group and from 1 to 20 carbon atoms in said alkyl radical with phosphorus pentasulfide at temperatures from 70° F. to 400° F. wherein the phosphorus pentasulfide-succinimide mol ratio is from 5:1 to 1:20 followed by (2) reacting the product of (1) with a polyalkylene polyamide at temperatures from 250° F. to 450° F. wherein the mol ratio of poly-amine to succinimide is from 0.5:1 to 1:1, said poly-alkylene polyamine being of the formula



wherein R is selected from the group consisting of ethylene and propylene and x is a number from 1 to 10.

2. The lubricating oil composition of claim 1 wherein said polyamine is tetraethylene pentamine.

3. The lubricating oil composition of claim 1 wherein said succinimide is reacted with said phosphorus pentasulfide at temperatures from 175° F. to 250° F., and said

10 phosphorus pentasulfide-succinimide product is reacted with said polyalkylene polyamide at temperatures from 280° F. to 350° F.

4. The lubricating oil composition of claim 3 wherein 5 said product is present in amounts from 0.1 to 15% by weight.

5. The lubricating oil composition of claim 4 wherein said phosphorus pentasulfide-succinimide mole ratio is from 1:1 to 1:4.

References Cited by the Examiner

UNITED STATES PATENTS

|           |       |                 |          |
|-----------|-------|-----------------|----------|
| 2,733,235 | 1/56  | Cross et al.    | 252—32.7 |
| 2,773,862 | 12/56 | Musselman       | 252—32.7 |
| 3,018,247 | 1/62  | Anderson et al. | 252—32.7 |

DANIEL E. WYMAN, Primary Examiner.

UNITED STATES PATENT OFFICE  
CERTIFICATE OF CORRECTION

Patent No. 3,185,647

May 25, 1965

Robert G. Anderson et al.

It is hereby certified that error appears in the above numbered patent requiring correction and that the said Letters Patent should read as corrected below.

Column 1, lines 67 to 72, for that portion of the formula reading



column 3, line 73, for "provided" read -- provide --; column 5, line 6 and column 6, line 2, for "polyamide", each occurrence, read -- polyamine --.

Signed and sealed this 19th day of October 1965.

(SEAL)

Attest:

ERNEST W. SWIDER  
Attesting Officer

EDWARD J. BRENNER  
Commissioner of Patents

UNITED STATES PATENT OFFICE  
CERTIFICATE OF CORRECTION

Patent No. 3,185,647

May 25, 1965

Robert G. Anderson et al.

It is hereby certified that error appears in the above numbered patent requiring correction and that the said Letters Patent should read as corrected below.

Column 1, lines 67 to 72, for that portion of the formula reading



column 3, line 73, for "provided" read -- provide --; column 5, line 6 and column 6, line 2, for "polyamide", each occurrence, read -- polyamine --.

Signed and sealed this 19th day of October 1965.

(SEAL)

Attest:

ERNEST W. SWIDER  
Attesting Officer

EDWARD J. BRENNER  
Commissioner of Patents